

## UNITED STATES PATENT OFFICE.

PIERRE GIRIN, OF PARIS, FRANCE, ASSIGNOR TO SOCIETE ANONYME DE COMMENTRY  
FOURCHAMBAULT & DECAZEVILLE, OF PARIS, SEINE, FRANCE.

## ALLOY.

No Drawing.

Application filed April 16, 1919. Serial No. 290,600.

*To all whom it may concern:*

Be it known that I, PIERRE GIRIN, a citizen of the Republic of France, residing in Paris, Department of the Seine, France, 5 have invented a certain new and useful Alloy, of which the following is a specification.

It has long been known that the brittleness of ordinary and special steels increases 10 very rapidly as the temperature falls below the ordinary temperature. Thus during very severe winters there is an increase in the number of accidental breakages of railway rails and carriage axles.

15 When the extreme temperatures of liquefied permanent gases are attained, iron and steel are very brittle and break at the least shock, like glass.

This property of iron and steel has for 20 long been a serious obstacle in the construction of machines required to operate at very low temperatures, so that parts more particularly concerned in the running of the machine are liable to be broken by shocks 25 more or less violent. This is particularly the case in machines for liquefying air by reversible expansion with external work (the Claude system); in this case the valves of the motor in which the expansion occurs 30 should be devoid of brittleness at the working temperature, which may be below  $-180^{\circ}$  centigrade.

The present invention relates to an alloy 35 of iron, nickel and manganese, which may contain carbon, chromium, copper, cobalt, titanium or vanadium, which alloy at the lowest temperatures (even at  $-200^{\circ}$  centigrade) is completely devoid of brittleness, while at the same time it has a high elastic 40 limit and mechanical strength.

One may take as an example an alloy containing nickel 40-70 per cent, manganese 0.8-5 per cent, iron the rest.

An example of a definite alloy having a 45 composition between these limits is one containing Ni 55 per cent, Mn 2 per cent, Fe 43 per cent.

Without inconvenience from the point of 50 view of brittleness and for the purpose of realizing some particular accessory quality relating, for instance, to dilatation, electrical properties, or elastic or mechanical properties, the content of nickel or manganese may be varied between the limits indicated. For example, an alloy containing

Ni 58, Mn 2, Fe 40 has the expansion of iron, and one containing Ni 46, Mn 1, Fe 53 an expansion equal to that of ordinary glass.

The tensile strength and the modulus of elasticity of an alloy having a certain composition may be brought to any value desired between certain limits. Thus there may be introduced one or several additional elements:—carbon up to 1 per cent, chromium up to 5 per cent, copper up to 10, 65 cobalt up to 10 per cent, so that the field of physical and mechanical constants may be still further enlarged.

Moreover, the addition of 0.2-1 per cent of vanadium, 0.1 to 0.5 per cent of titanium 70 has a very favourable action on the quality of the alloy and the facility with which it can be made. The amounts indicated for the additional elements are substituted for the corresponding amounts of iron. 75

Such an alloy has all the satisfactory mechanical properties of reversible ferro-nickel and the composition of it renders possible any irreversible transformation and any alteration due to the action of cold. At 80 the boiling point of nitrogen, namely  $-195^{\circ}$  C., the elastic limit may vary between 35 and 45 kilos per square millimeter and the tensile strength between 65 to 75 per square millimeter. 85

The resilience, measured on the Frémont system, attains 50 kilos at ordinary temperature and preserves this value up to  $-195^{\circ}$  C. For the purpose of comparison it may be added that the softest iron exhibits at 90 this low temperature only 1-2 kilos.

This new alloy is non-oxidizable and is practically unattacked by sulphuric acid of all concentrations: for example, cold sulphuric acid of 28° Baumé dissolves .2m/mg 95 per cm<sup>2</sup> of the alloy, in 6 hours. If desired it may be given the coefficient of expansion of cast iron or steel so that an exact adjustment made at ordinary temperature between two parts, one of the present alloy 100 and the other of iron or steel is maintained at low temperatures. Finally, parts made of this alloy may be subjected to repeated shocks without deformation, cracking or flattening. 105

Having thus described the nature of the said invention and the best means I know of carrying the same into practical effect, I claim:—

1. An article of manufacture for use in 110

the liquefaction of gases which retains its resiliency and mechanical strength at the low temperatures realized in the liquefaction of gases, composed of a nickel-ferrous alloy comprising 40 to 70% of nickel, 0.8 to 5% of manganese, and the principal portion of the remainder of iron.

2. An article of manufacture which retains its resiliency and mechanical strength

at industrially low temperatures such as are realized in the liquefaction of gases, composed of a nickel-ferrous alloy comprising 40 to 70% of nickel, 0.8 to 5% of manganese, and the rest of iron.

In witness whereof, I have hereunto signed my name.

PIERRE GIRIN.